

## UNITED STATES PATENT OFFICE

2,039,082

PREPARATION FOR PROTECTING AND  
SEALING WOUNDS AND METHOD OF  
MANUFACTURING THE SAMEKarl Jungmann, Aussig-on-the-Elbe,  
CzechoslovakiaNo Drawing. Application December 17, 1934,  
Serial No. 757,963. In Germany March 25,  
1931

6 Claims. (Cl. 167—58)

This invention relates to pulverulent preparations for protecting and sealing wounds, and more particularly for use as a mechanically acting hemostatic, and relates further to a method 5 of manufacturing such preparations. It is an object of the invention to provide a preparation which is capable, when brought in contact with the fluid discharge from the wound, to absorb the same and to form a plaster-like coating which 10 mechanically seals the wound. A further object is to provide a preparation, which through the formation of a tough elastic skin in the moment of application to bleeding wounds, is capable of withstanding the pressure of the blood (within 15 certain limits), so that further hemorrhage is checked. Further objects of the invention will become apparent in the course of the ensuing description.

The invention is based upon the discovery that 20 it is necessary, for the purpose of mechanical blood stanching by the formation of a seal, to employ pulverulent swelling substances, such as insoluble kinds of gum exemplified by various varieties of tragacanth, and ground seed kernels 25 of the carob bean, having the property, at normal temperatures up to body-temperature, of forming immediately, that is to say within a few, generally less than 5, seconds after contact with the fluid discharge, coherent and elastic jellies 30 which will withstand the pressure of this fluid.

The expression "gum tragacanth" is intended 35 to cover all of the various gums known by that name and including the various species and varieties of *Astragalus*, and the various varieties and species of *Sterculia* and *Cochlospermum gossypium*. Gum from *Sterculia* is sometimes known as Karaya gum, but according to the British Pharmaceutical Codex 1923 it is also called Indian tragacanth.

In some cases, it is desirable that the pulverulent 40 swelling substances used have the property of permanently taking up the discharge from the wound, while swelling and forming jellies. For the attainment of this object there are two factors of decisive importance, namely first the swelling velocity of the initial pulverulent substances, which in its turn has to do inter alia with their capacity for becoming wetted and 45 secondly the firmness of the gels formed. I have now found that the swelling velocity of powders capable of swelling, and more still the firmness 50 of the jellies formed from these powders on contact with water or aqueous liquids such as blood, is dependent to a very considerable extent on 55 the grain size of the powder employed. In order

to obtain the optimum effect it is necessary that the pulverulent substances used do not contain portions of a grain size exceeding a certain upper limit. I have found that the pulverulent substances used, if they are to exhibit the required 5 properties, must be free from particles which are retained by a screen No. 35 (width of opening 0.500 mm.). Such powders are still better suited that in addition are free from particles which are retained by a screen No. 70 (width of 10 opening 0.210 mm.). I have further found that it is of advantage to use pulverulent substances which are also free from constituents of the fineness of dust, preferably from portions of a grain size to pass through a screen No. 200 (width 15 of opening 0.074 mm.), and better still from portions of a grain size to pass through a screen No. 140 (width of opening 0.105 mm.).

Any partial fraction lying anywhere between the above given limits may be separated out and 20 used for the purpose in view.

For the purpose of producing powder of this 25 nature, the starting materials are comminuted, for example in a mill of close set, mortar, or the like, after which at least the coarse particles, but preferably also the particles of the fineness of dust, are removed. For the separating out of the 30 particles to be eliminated there can be employed all the usual methods, such as screening, wind sifting, and the like. It is simplest to dress the 35 powdered material according to grain sizes, by screening. The coarse particles are eliminated by sieving out on a screen No. 35 or any other screen between No. 35 and No. 70. The finest particles are then preferably eliminated by sieving out on a screen No. 200. It is, however, of 40 advantage, as mentioned above, to separate out still coarser particles than those corresponding to screen No. 200. For this purpose for example a screen No. 140 or any screen between Nos. 140 and 200 is taken. The sieve designation here 45 used is that of the U. S. Standard (International Critical Tables of Numerical Data, Physics, Chemistry and Technology, prepared under the auspices of the International Research Council and the National Academy of Sciences by the National Research Council of the U. S. of Am. vol. II, page 329).

The capacity of the powder of being wetted 50 and thus its velocity of swelling, and, moreover, the firmness of the gels formed on contact with aqueous liquids may also be considerably increased by subjecting the powder to a heat treatment under such conditions, as regards temperature and duration of the heat action, that a 55

noticeable change of the color, generally a change to yellow or brown, takes place. This change of the color usually sets in after a period of one hour when heating the powder up to 100 or 120° C., and already after a shorter period when heating to higher temperatures. This heat treatment may be effected before dressing the powder to remove the constituents retained by sieve No. 35. But it is also possible to subject the powder already dressed to this heat treatment.

If pulverulent substances according to the present invention be employed these substances, when brought in contact in suitable quantities with the liquid discharge, at body-temperature, will swell within a very short time, generally within less than five seconds, and form an elastic and firm jelly constituting an immediate and firmly adhering protective cover and seal of the wound.

The swelling pulverulent substances can be sterilized in a known manner, for example by treatment with antiseptically active substances, preferably with readily evaporating substances of the nature of chloroform, toluol, and the like, or with other known disinfectants such as trypano-

25 flavin, bismuth salts, iodoform and the like. If the sterilizing is effected by the application of heat, the heat treatment described above for the purpose of increasing the capacity of the powder of being wetted may be combined in a simple manner with the sterilization, by carefully heating the swelling substances for several hours, for example in a thin layer or with agitation, to a temperature in the neighbourhood of 100° C., whereupon the temperature is increased until the water is practically driven off, which is often the case at 120° C. The powder thus treated is now further heated in a closed vessel, for example at temperatures of 120° to 130° C., until the desired capacity of being wetted and the change in color which depend on each other, are attained. The powder becomes at the same time sterile.

There can also be added to the inert swelling powders substances of specific efficacy, such as styptics, disinfectants, or analgetics, either singly or in combination.

The preparations obtained in accordance with the invention can be sold either in the form of a loose powder to be strewn or dusted on to wounds, or can be incorporated in carrier materials such as surgical dressing fabric, cotton-wool, lint, paper, plasters, and the like. If a carrier material such as cotton-wool is used the fibrous material is embedded in the gel formed from the powder in contact with the fluid discharge.

In contradistinction to the usual surgical dressing fabrics or the chemical acting agents for treating wounds or blood stanching, which either do not prevent with certainty the penetration of microbes into the wound or hinder the discharge of secretions from the wound, the swelling powders described are capable of absolutely sealing the wounds and at the same time binding the secretion by absorbing it. While swelling, they also permit stanching rapidly and reliably haemorrhages which hitherto have been regarded as incapable of being stanched such as for example haemorrhages following incisions of the liver.

#### Examples

(1) 1000 grams of ground seeds of the carob bean are first freed from the grained particles which are too coarse, with the aid of screen No. 70, and then from the particles of the fineness

of dust by sieving on a screen No. 140. In this latter screen there remain about 550 grams. This sieved fraction is spread out in a thin layer on glass dishes, and heated for 2 hours at about 110° C. in the drying chamber. The product assumes a faintly yellow color in the course of heating. After this drying process the powder is placed in a bottle which is closed with a plug of cotton-wool and heated in the drying chamber for 3 hours at 130° C. The color of the powder will now change to a brownish color and becomes sterile.

(2) The sieved fraction of 550 grams weight obtained in accordance with Example (1) is uniformly sprinkled with 50 ccs. of a 10% alcoholic solution of trichlore-isobutyl alcohol (chloreton), and the alcohol allowed to evaporate.

(3) The sieved fraction of 550 grams weight obtained in accordance with Example (1) is sprinkled, if desired after heating, with 50 ccs. of a 10% solution of iodine in chloroform which is then allowed to evaporate. The disappearance of the chloroform is visible by the iodine changing color from reddish-violet to brown. Tincture of iodine can also be employed, to obtain a strongly antiseptic product.

(4) 1000 grams weight of gum tragacanth are comminuted and heated in the heating chamber for 2½ hours to 140° C. The product changes its color after a short time to a faintly yellow color and becomes gradually brownish. The heat treated powder is now sieved on a screen No. 50, and the constituents passing this screen are freed from the dust-like particles by screening on a screen No. 170.

#### What I claim is:

1. A hemostatic preparation capable of swelling when in contact with aqueous liquids for mechanically sealing and protecting bleeding wounds comprising a powder of a gum selected from the class consisting of tragacanth and carob bean seed kernels, the said powder consisting of particles mainly of such grain sizes as pass through screen No. 35 and are retained by screen No. 200, and forming with the wound secretions a firm coherent coating mass which adheres strongly to the flesh of the wound.

2. A hemostatic preparation capable of swelling when in contact with aqueous liquids for mechanically sealing and protecting bleeding wounds comprising a powder of a gum selected from the class consisting of tragacanth and carob bean seed kernels, the said powder consisting of particles mainly of such grain sizes as pass through screen No. 70 and are retained by screen No. 140, and forming with the wound secretions a firm coherent coating mass which adheres strongly to the flesh of the wound.

3. A hemostatic preparation capable of swelling when in contact with aqueous liquids for mechanically sealing and protecting bleeding wounds comprising a substantially dehydrated powder of a gum selected from the class consisting of tragacanth and carob bean seed kernels, the said powder consisting of particles mainly of such grain sizes as pass through screen No. 70 and are retained by screen No. 140, and forming with the wound secretions a firm coherent coating mass which adheres strongly to the flesh of the wound.

4. A hemostatic preparation capable of swelling when in contact with aqueous liquids for mechanically sealing and protecting bleeding wounds comprising a substantially dehydrated

- powder of a gum selected from the class consisting of tragacanth and carob bean seed kernels, the said powder consisting of particles mainly of such grain sizes as pass through screen 5 No. 35 and are retained by screen No. 200, and forming with the wound secretions a firm coherent coating mass which adheres strongly to the flesh of the wound.
5. A process of producing a preparation capable of swelling when in contact with aqueous liquids, for protecting and sealing wounds which consists in comminuting a gum selected from the class consisting of tragacanth and carob bean seed kernels to a powder and dressing the said powder to remove coarse grains.
6. A process of producing a preparation capable of swelling when in contact with aqueous liquids, for protecting and sealing wounds which consists in comminuting a gum selected from the class consisting of tragacanth and carob bean seed kernels to a powder, dressing the said powder to remove coarse grains and thereafter subjecting the said powder to a heat treatment for such a 5 period and sufficient to substantially dehydrate the same.

KARL JUNGMANN.